

Patented Jan. 10, 1939

2,143,205

## UNITED STATES PATENT OFFICE

2,143,205

## ARTIFICIAL SILK

Richard Müller, Berlin-Schöneberg, and Alfred Lübbe, Mannheim-Waldhof, Germany, assignors to C. F. Boehringer & Soehne G. m. b. H., Mannheim-Waldhof, Germany

No Drawing. Application February 7, 1934, Serial No. 710,113. In Germany February 15, 1933

1 Claim. (Cl. 18—54)

The present invention relates to the production of artificial silk and similar artificial products including ribbons, films etc., more especially from cellulose esters of carboxylic acids, and one of its objects is the production of products of this kind, which are mechanically stronger than similar products hitherto produced.

It has been found that if solutions of cellulose esters of carboxylic acids are spun in accordance with the wet spinning process, the mechanical strength of the threads, ribbons, films or the like is increased if the coagulation of the esters takes place in precipitating liquors kept at a low temperature. Already at a temperature approaching 0° C., for instance at +2° a stronger product is obtained and if the temperature is lowered further, for instance to -10°, -20° and -40° and further down a further increase of strength is obtained.

In order to demonstrate the influence of low temperatures of the order mentioned above on the strength of the artificial thread, ribbon or film, we will now proceed to give the results of some of many comparative tests made with different esters and precipitating liquors at different temperatures.

## Example 1

A fibriform cellulose triacetate washed and dried in the usual manner was dissolved in a mixture formed of 95 parts by volume methylene chloride and 5 parts alcohol, the concentration of the solution used in the different tests being shown in the following schedule in cubic centimetres of the solvent per gram of the ester. The solutions were spun in the manner well known in the wet spinning process with a draft velocity of 10 to 20 metres per minute through a nozzle formed with 36 holes, each 0.08 millimetre in diameter, the precipitating liquid being ether and the threads obtained being collected on bobbins or in a centrifugal.

| Temperature of precipitating bath | Concentration of spinning solution | Titer of single thread: deniers | Elongation in percent | Strength of single thread in grams per denier |         |  |
|-----------------------------------|------------------------------------|---------------------------------|-----------------------|-----------------------------------------------|---------|--|
|                                   |                                    |                                 |                       |                                               | Degrees |  |
| +20                               | 1:9                                | 3.0                             | 22                    | 1.34                                          |         |  |
| +20                               | 1:9                                | 2.2                             | 22                    | 1.33                                          |         |  |
| +20                               | 1:11                               | 2.7                             | 26                    | 1.30                                          |         |  |
| +20                               | 1:11                               | 2.0                             | 26                    | 1.31                                          |         |  |
| +2                                | 1:9                                | 3.0                             | 17                    | 1.51                                          |         |  |
| +2                                | 1:9                                | 2.2                             | 16                    | 1.56                                          |         |  |
| 0                                 | 1:9                                | 3.5                             | 18                    | 1.60                                          |         |  |
| 0                                 | 1:9                                | 2.2                             | 15                    | 1.59                                          |         |  |
| -10                               | 1:9                                | 3.7                             | 16                    | 1.67                                          |         |  |
| -10                               | 1:9                                | 3.0                             | 14                    | 1.70                                          |         |  |
| -20                               | 1:11                               | 3.2                             | 16                    | 1.83                                          |         |  |
| -20                               | 1:11                               | 2.4                             | 15                    | 1.80                                          |         |  |
| -30                               | 1:13                               | 2.7                             | 15                    | 2.7                                           |         |  |
| -30                               | 1:13                               | 2.0                             | 14.5                  | 2.06                                          |         |  |
| -40                               | 1:13                               | 3.5                             | 12.5                  | 2.23                                          |         |  |
| -40                               | 1:13                               | 1.8                             | 10                    | 2.34                                          |         |  |

## Example 2

In a similar manner and with the same nozzle a similar solution of cellulose triacetate was precipitated in toluene.

| Temperature of precipitating bath | Concentration of spinning solution | Titer of single thread: deniers | Elongation in percent | Strength of single thread in grams per denier |  |
|-----------------------------------|------------------------------------|---------------------------------|-----------------------|-----------------------------------------------|--|
| Degrees                           |                                    |                                 |                       |                                               |  |
| -17                               | 1:16                               | 2.08                            | 20.5                  | 1.10                                          |  |
| -17                               | 1:16                               | 1.46                            | 20.5                  | 1.09                                          |  |
| -30                               | 1:16                               | 2.06                            | 15.5                  | 1.68                                          |  |
| -30                               | 1:16                               | 1.45                            | 14                    | 1.68                                          |  |
| -40                               | 1:16                               | 2.08                            | 15                    | 1.84                                          |  |
| -40                               | 1:16                               | 1.44                            | 14                    | 1.82                                          |  |
| -50                               | 1:16                               | 1.97                            | 9.5                   | 2.03                                          |  |

## Example 3

A solution of a cellulose triacetate hydrolyzed to the extent of containing 59.7% acetic acid and dissolved in methylene chloride-alcohol (95:5) was spun and precipitated in ether.

| Temperature of precipitating bath | Concentration of spinning solution | Titer of single thread: deniers | Elongation in percent | Strength of single thread in grams per denier |  |
|-----------------------------------|------------------------------------|---------------------------------|-----------------------|-----------------------------------------------|--|
| Degrees                           |                                    |                                 |                       |                                               |  |
| +14                               | 1:11                               | 3.36                            | 27                    | 1.27                                          |  |
| +14                               | 1:11                               | 1.87                            | 26                    | 1.36                                          |  |
| -20                               | 1:11                               | 3.2                             | 17.5                  | 1.50                                          |  |
| -20                               | 1:11                               | 2.6                             | 17.0                  | 1.59                                          |  |
| -40                               | 1:11                               | 3.0                             | 13                    | 1.84                                          |  |
| -40                               | 1:11                               | 2.45                            | 13                    | 1.92                                          |  |

## Example 4

A cellulose diacetate dissolved in the same solvent mixture was precipitated in ether.

| Temperature of precipitating bath | Concentration of spinning solution | Titer of single thread: deniers | Elongation in percent | Strength of single thread in grams per denier |  |
|-----------------------------------|------------------------------------|---------------------------------|-----------------------|-----------------------------------------------|--|
| Degrees                           |                                    |                                 |                       |                                               |  |
| +16                               | 1:11                               | 4.34                            | 26.5                  | 0.80                                          |  |
| +16                               | 1:11                               | 3.22                            | 21.5                  | 0.84                                          |  |
| -20                               | 1:11                               | 3.41                            | 23                    | 1.25                                          |  |

## Example 5

A cellulose acetobutyrate containing 8% butyric acid and dissolved in a mixture of 95 parts methylene chloride and 5 parts alcohol was spun and precipitated in ether.

| Temperature of precipitating bath | Concentration of spinning solution | Titer of single thread: deniers | Elongation in percent | Strength of single thread in grams per denier |  |
|-----------------------------------|------------------------------------|---------------------------------|-----------------------|-----------------------------------------------|--|
| Degrees                           |                                    |                                 |                       |                                               |  |
| +18                               | 1:11                               | 2.88                            | 26.5                  | 1.13                                          |  |
| -40                               | 1:11                               | 2.87                            | 17                    | 1.64                                          |  |
| -50                               | 1:11                               | 3.09                            | 15                    | 1.79                                          |  |

Similarly as the cellulose esters mentioned above also other simple cellulose esters, such as the formates, propionates or butyrates or mixed cellulose esters, such as the acetoformates, aceto-propionates or acetobutyrate, as well as the products obtained by subjecting the primary esters to a more or less far reaching hydrolytic decomposition may be subjected to the new process, the most suitable solvents being used in each individual case.

We have found that when proceeding in accordance with this invention, i. e. introducing the cellulose ester solution into a coagulating liquid cooled down to at least +2° C., we may also use, as solvents for the esters, solvents or solvent mixtures which are known to be unsatisfactory when coagulation is effected at a higher temperature. Thus for instance solutions of mixed esters in a mixture of 95 parts ethylene chloride and 5 parts ethyl alcohol or in a mixture of 23 parts acetone and 10 parts dioxan can be coagulated and yield strong threads in a coagulation liquid cooled down to at least +2° C. and preferably to -20° C.

Instead of ether and toluene also other precipitants, such as benzine, petroleum, cyclohexan and others may serve for precipitating the esters.

Instead of spinning solutions of isolated cellulose esters, it is also possible in some cases to

directly spin the solutions obtained in the production of the cellulose esters, as is known in the spinning processes carried through at higher temperatures.

It will be interesting to know that when proceeding in accordance with the present invention, the precipitating liquors can be used much longer without being regenerated, than can be done in a process operating at higher temperature, because the precipitating effect is preserved at the low temperatures even if the liquor is highly diluted by the solvents.

Operation at low temperature also counteracts the losses encountered when using readily volatile liquids for precipitating the esters.

Various changes may be made in the details disclosed in the foregoing specification without departing from the invention or sacrificing the advantages thereof.

We claim:—

The method of coagulating solutions of carboxylic acid esters of cellulose comprising introducing the solutions into a neutral organic coagulating liquid having a melting point below +2° C. and cooled below +2° C.

RICHARD MÜLLER.  
ALFRED LÜBKE.